# EUROPEAN PATENT SPECIFICATION

(11) **EP 3 553 199 B1**
(45) Date of publication and mention of the grant of the patent: **08.07.2020**
(21) Application number: 19153314.0
(22) Date of filing: 23.01.2019
(51) Int. Cl.: C22C 49/00, C22C 49/02, C22C 49/14

(54) **A METHOD OF PREPARING MAGNESIUM-ZINC-YTTRIUM QUASICRYSTAL AND BORON CARBIDE MIXED REINFORCED MAGNESIUM-BASED COMPOSITE MATERIAL**
VERFAHREN ZUR HERSTELLUNG EINES MAGNESIUM-ZINK-YTTRIUM-QUASIKRISTALL UND BORCARBID-GEMISCHTEN VERSTÄRKTEN MAGNESIUM-BASIERTEN KOMPOSITMATERIALS
PROCÉDÉ DE PRÉPARATION DE MATÉRIAU COMPOSITE À BASE DE MAGNÉSIUM RENFORCÉ MÉLANGE PAR DU MAGNÉSIUM-ZINC-YTTRIUM QUASI-CRISTAL ET DU CARBURE DE BORE

(30) Priority: 13.04.2018 CN 201810328616
(43) Date of publication of application: 16.10.2019
(73) Proprietor: North University of China, Taiyuan City, Shanxi 030051 (CN)
(72) Inventor: Zhao, Yuhong, Taiyuan city, Shanxi 030051 (CN); Tian, Jinzhong, Taiyuan city, Shanxi 030051 (CN); Hou, Hua, Taiyuan city, Shanxi 030051 (CN); Wen, Zhiqin, Taiyuan city, Shanxi 030051 (CN); Chen, Liwen, Taiyuan city, Shanxi 030051 (CN); Guo, Huijun, Taiyuan city, Shanxi 030051 (CN)
(74) Representative: Global IP Europe Patentanwaltskanzlei

(56) References cited:
- US-A1- 2016 230 251
- US-A1- 2016 355 913

## Description

### CROSS-REFERENCE TO RELATED APPLICATION

The application claims priority to Chinese Application No. 201810328616.X, filed on April 13, 2018.

### BACKGROUND

### Field of Invention

The present invention relates to a method of preparing magnesium-zinc-yttrium quasicrystal and boron carbide mixed enforced Mg-based composite materials, which belong to the technical area of preparing and applying the non-ferrous metal materials.

### Background of the Invention

The magnesium alloy materials have widely applied in the automobile and aerospace area for it they are characterized in low density, high specific strength, excellent shock resistance, strong electromagnetic shielding capability and easy processing. However, the application of magnesium alloy in the industrial area is restricted for its low hardness, low anti-tensile strength and poor corrosion resistance. The Chinese patent CN 102618766B discloses a method of producing a quasicrystal enhanced Mg-Zn-Y alloy by means of conventional melting and subsequent thermal treatment.

As the quascicrystal has high hardness, high elastic modules, low expansion coefficient and excellent corrosion resistance, it is extremely suitable to be used as the enhance phase of the magnesium alloy and can efficiently improve the mechanical property of the magnesium alloy. The boron carbide particles are of great application potential for they have low density, excellent chemical stability, abrasive resistance and can be evenly distributed in the magnesium substrate with a stable interface. However, mixed particles reinforced Mg-based composite materials are still in the research phase and the process technology needs to be improved.

### SUMMARY

### Invention Object

The present invention is done based on the situations introduced by the background art and aims at improving the mechanical property of the magnesium alloy by adopting the magnesium alloy as the substrate, the endogenous magnesium-zinc-yttrium quasicrystal and boron carbide as the reinforced phase, via smelting in the vacuum medium frequency induction melting furnace and then squeezing casting to prepare magnesium-zinc-yttrium quasicrystal and boron carbide mixed reinforced Mg-based composite materials.

### Technical Solution

Chemical materials used in the present invention are: magnesium, zinc, magnesium yttrium interalloy, boron carbide, zinc oxide, talcum powder, water glass, deionized water, aluminum foil, absolute alcohol, argon, their amounts used in the composition are: (measured in gram, milliliter and centimeter³):

| | | |
|---|---|---|
| magnesium | Mg | 4127g±0.1g |
| Zinc | Zn | 784g±0.1g |
| magnesium yttrium interalloy | Mg₈₉Y₁₁ | 571g±0.1g |
| boron carbide | B₄C | 300g±0.1g |
| zinc oxide | ZnO | 80g±1g |
| talcum powder | Mg₃Si₄O₁₀](OH)₂ | 50g±1g |
| water glass | Na₂SiO₃·9H₂O | 25g±1g |
| deionized water | H₂O | 1000mL±50mL |
| aluminum foil | Al | 300mm×0.5mm×300mm |
| absolute alcohol | C₂H₅OH | 3500mL ±50mL |
| argon | Ar | 800000cm³±100 cm³ |

the preparation method comprises:
(1) preparing the casting mold
   the open-close type squeeze casting mold is manufactured by hot working dies steel with a rectangle cavity, wherein the size of the cavity is 200mm×160mm×90mm and the surface roughness of the cavity is Ra 0.08-0.16µm;
(2) preparing the coating agent
   weighing out zinc oxide 80g±1g, talcum powder 50g±1g, water glass 25g±1g, measuring out deionized water 300mL±1mL, adding zinc oxide 80g±1g, talcum powder 50g±1g, water glass 25g±1g and deionized water 300mL±1mL into the mixinghollander and stirring them to obtain the coating agent presenting as viscous liquid, wherein the stirring speed is 50r/min, stirring time is 80min.
(3) pre-treating the boron carbide particles
   ①ball milling: weighing boron carbide 300g±0.1g, putting it into the ball mill tank of the ball mill and ball milling it to obtain fine powder with a particle size ≤9µm, wherein the ball milling speed is 80r/min, the ball milling time is 3h;
   ②ultrasonic dispersion washing: putting the fine powder after ball milling into a beaker and then adding absolute alcohol 500mL±1mL, mixing;
      putting the beaker into an ultrasonic disperser and doing the ultrasonic dispersion washing to obtain the mixing liquid, wherein the ultrasonic frequency is 60kHz and the ultrasonic dispersion time is 80min;
   ③filtration: putting the mixing liquid into the cloth funnel of the filter bottle, filtering it with a microporous membrane, removing the supernatant, and keeping the filter cake;
   ④drying and oxidation treatment: putting the filter cake into the thermal treatment furnace, conducting the drying and high temperature oxidation treatment, obtaining the boron carbide fine powderafter drying, wherein the drying and oxidation temperature is 500°C and the drying and oxidation time is 2h;
(4)pre-treating the magnesium, zinc and magnesium yttrium interalloy and the open-close type squeeze casting mold
   ①mechanically cutting the magnesium, zinc and magnesium yttrium interalloy into patches, wherein the size of the patch is ≤30mm×30mm×10mm;
   ②washing the surface of the magnesium, zinc and magnesium yttrium interalloy with absolute alcohol and then putting it into the vacuum drying oven after washing, wherein the drying temperature is 100°C, the vacuum degree is 2 Pa and the drying period is 30min;
   ③wrapping the boron carbide with aluminum foil, putting it into the vacuum drying ovenand drying, wherein the drying temperature is 100°C, the vacuum degree is 2 Pa and the drying period is 60min;
      pre-heating the open-close type squeeze casting mold and coating the prepared coating agent on the inner surface of the mold cavity, wherein the thickness of the coating agent is 1mm; after the coating is completed, putting the open-close type squeeze casting mold into the heating furnace and preheating, wherein the pre-heating temperature is 150°C and the pre-heating time is 1h;
(5) smelting of the magnesium alloy
   smelting of the magnesium alloy is conducted in the vacuum medium frequency induction melting furnace and completed by processes of medium frequency induction heating, vacuumizing, bottom blowing argon and mechanical stirring;
   ①opening the vacuum medium frequency induction melting furnace and clearing the internal part of the graphite melting crucible to make the internal part of the crucible clean;
   ②weighing magnesium block 4127g±0.1g, zinc block 784g±0.1g and magnesium yttrium interalloy block 571g±0.1g and putting them in the bottom of the crucible;
   ③closing the vacuum medium frequency induction melting furnace and getting it sealed;
      turning on the vacuum pump and extracting the air within to allow the pressure within the furnace to reach 1Pa;
      turning on the heater of the medium frequency induction melting furnace to start the heating, wherein the heating temperature is 610°C±1°C;
   ④tuming on the argon bottom-blowing device to feed argon into the crucible, wherein the speed of the argon bottom-blowing is 200cm³/min; adjusting the pressure within the furnace to maintain the pressure within the furnace to be one bar pressure and it is regulated by the outlet valve;
   ⑤when the temperature of melt is 610°C±1°C, adding boron carbide fine powder with the vacuum feeding device; turning on the mechanical agitator, wherein the stirring speed is 20r/min and the stirring time is 10min;
   ⑥stopping the stirring and continuing the heating; when the temperature of melt reaches 730°C±1°C, turning off the mechanical agitator and the argon bottom blowing pipe, standing for 10 min to prepare for the casting;
(6) squeeze casting
   ①opening the vacuum medium frequency induction melting furnace, removing the slag on the surface of the melt in the crucible, casting the alloy melt into the cavity of the squeeze casting mold; turning on the squeeze casting machine and squeezing the metal melt by the punch, wherein the squeeze pressure is 250MPa and the hold time is 20s;
      the alloying reaction occurs during the solidification of Mg-Zn-Y quascicrystal and stable quascicrystal Mg₃Zn₆Y phase can be produced, wherein the reaction formula is $Mg + Zn + {Mg}_{89} {Y}_{11} + {B}_{4} C {\to }_{250 MPa}^{20 s} α - Mg + {Mg}_{3} {Zn}_{6} Y + {B}_{4} C$
      α-Mg : substrate magnesium phase
      Mg₃Zn₆Y : magnesium zinc yttrium quasicrystalline phase
   ②ejecting the cast and cooling it to 25°C in the air to produce the magnesium-zinc-yttrium quasicrystal and boron carbide mixed reinforced Mg-based composite material blocks;
(7)thermal treatment of the cast
   ①putting the magnesium-zinc-yttrium quasicrystal and boron carbide mixed reinforced Mg-based composite material blocks into the vacuum heat treatment furnace for thermal treatment, wherein the temperature of the thermal treatment is 420°C, the vacuum degree is 2Pa, and the time of thermal treatment is15h; and then putting the cast into warm water of 50°C fastly, quenching treatment, wherein the quenching time is 20s;
   ②putting the cast after quenching into the heat treatment furnace for aging treatment at 200°C for 8h; and then stopping the heating and cooling it to 25°C in the heat treatment furnace;
(8) cleaning, detecting, analyzing and characterizing
   cleaning the surface of the cast to make it clean; detecting, analyzing and characterizing the microstructure and mechanical property;
   analyzing the metallographic structure with an optical microscope;
   conducting the tensile strength and hardness test with universal tensile testing machine and a hardness tester;
   conducting the fracture morphology analysis with a scanning electron microscope;
   conducting XRD analysis with X ray diffractometer;
   conclusion: magnesium-zinc-yttrium quasicrystal and boron carbide mixed reinforced Mg-based composite materials are rectangle blocks, wherein the tensile strength thereof is 315MPa, the elongation is 7%, the hardness reaches 108Hv.

### Beneficial effects

Compared with the background arts, the present invention has prominent advantages. Based on the situations that the Mg-based composite materials have poor mechanical properties, in the present invention, magnesium-zinc-yttrium quasicrystal and boron carbide mixed reinforced Mg-based composite materials are prepared by adopting the magnesium alloy as the substrate, the endogenous magnesium-zinc-yttrium quasicrystal and boron carbide as the reinforced phase, via smelting in the vacuum medium frequency induction melting furnace, protection of bottom blowing argon, mechanical stirring, squeeze casting and heat-treatment. The preparation method has advanced process and strict procedures, wherein the data is accurate and detailed, and the prepared Mg-based composite materials have 315MPa tensile strength, 7% elongation, 108Hv hardness, making it an advanced preparation method of mixed reinforced Mg-based composite materials.

### BRIEF DESCRIPTION OF THE DRAWINGS

Figure 1 is the smelting state diagram of the Mg-based composite materials;
Figure 2 is the metallographic structure diagram of Mg-based composite materials;
Figure 3 is the fracture topography of Mg-based composite materials;
Figure 4 is is X-ray diffraction intensity spectrum of Mg-based composite materials;
   As shown in the figures, markers for the figures are listed as follow:
   1. vacuum medium frequency induction melting furnace, 2. furnace base, 3. furnace chamber, 4. outlet pipe, 5. outlet valve, 6. worktable, 7. graphite melting crucible, 8. medium frequency induction heater, 9. alloy melt, 10. argon, 11. bottom blow motor, 12. bottom blow pipe, 13. vacuum pump, 14. vacuum pipe, 15. argon bottle, 16. argon pipe, 17. argon valve, 18. electric cabinet, 19. display screen, 20. indicator light, 21. power switch, 22. medium frequency induction heating controller, 23. bottom blow motor controller, 24. vacuum pump controller, 25. first cable, 26. second cable, 27. feed pipe, 28. feed valve, 29. mechanical agitator.

### DETAILED DESCRIPTION OF THE EMBODIMENTS

Now the present invention will be further described in combination with the figures:
As shown in Figure 1, it shows the smelting state diagram of the Mg-based composite materials, wherein the location and connection relationship of each part should be correct and the ratio is conducted according to the amount and the process should be conducted according to the sequence.

The amount of the chemical materials used in the preparation of smelting is determined by the pre-configured scope, and they are measured in gram, milliliter and centimeter³.

The smelting of Mg-based composite materials is conducted in the vacuum medium frequency induction melting furnace, and finished by the process of mediate frequency induction heating, bottom blowing argon and mechanical stirring.

The vacuum medium frequency induction melting furnace is a vertical one. The bottom of the vacuum medium frequency induction melting furnace 1 is a furnace base 2, and the inside of the vacuum medium frequency induction melting furnace 1 is a furnace chamber 3; a worktable 6 is configured in the bottom of the furnace chamber 3 and a graphite melting crucible 7 is put on the worktable 6. The outside of the graphite melting crucible 7 is surrounded by the medium frequency induction heater 8 and the inside of the graphite melting crucible 7 is the alloy melt 9; an outlet pipe 4 is configured on the top right of the vacuum medium frequency induction melting furnace 1 and it is controlled by the outlet valve 5; the argon bottle 15 is configured on the top left of the vacuum medium frequency induction melting furnace 1 and an argon pipe 16 and an argon valve 17 are configured on the argon bottle 15. The argon pipe 16 is connected to the bottom blow motor 11. The bottom blow motor 11 is connected to the bottom blow pipe 12. The bottom blow pipe 12 communicates to the graphite melting crucible 7 through the furnace base 2 and worktable 6 and bottom blows the alloy melt 9; a vacuum pump 13 is configured in the bottom right of the furnace base 2 and communicates to the furnace chamber 3 through a vacuum pipe 14; a feed pipe 27, a feed valve 28 and a mechanical agitator 29 are configured on the top of the vacuum medium frequency induction melting furnace 1 and the feed pipe 27 and the mechanical agitator 29 extends to the graphite melt crucible 7 through the furnace top base.

A electric cabinet 18 is configured on the right of the vacuum medium frequency induction melting furnace 1 and a display screen 19, an indicator light 20, a power switch 21, a medium frequency induction heating controller 22, a bottom blow motor controller 23 and a vacuum pump controller 24 are configured on the electric cabinet 18; the electric cabinet 18 is connected to the medium frequency induction heater 8 through a first cable 25; The electric cabinet 18 is connected to the bottom blow motor 11 and a vacuum pump 13 through the second cable 26; the furnace cavity 3 is filled with argon 10.

As shown in Figure 2, it shows the metallographic structure diagram of Mg-based composite materials, wherein there are no defects such as inclusion and air holes in the metallographic structure diagram and the quascicrystal phase Mg₃Zn₆Y and boron carbide particles can be evenly distributed in particles.

As shown in Figure 3, it shows the fracture topography of Mg-based composite materials, wherein massive small dimples exist in the fracture topography and it demonstrates that it has excellent plasticity.

As shown in Figure 4, it shows X-ray diffraction intensity spectrum of Mg-based composite materials. In the figure, the ordinate is diffraction intensity index and the abscissa is the diffraction angle 2θ. It can be seen that mainly α-Mg substrate magnesium phase, Mg₃Zn₆Y quascicrystal phase and B₄C reinforced phase exist in Mg-based composite materials.

## Claims

1. A method of preparing a magnesium-zinc-yttrium quasicrystal and boron carbide mixed reinforced Mg-based composite materials, **characterized in that**, chemical materials used are: Magnesium, zinc, magnesium yittrium interalloy, boron carbide, zinc oxide, talcum powder, water glass which is Na₂SiO₃·9H₂O, deionized water, aluminum foil, absolute alcohol, argon, their amounts are:
| | | |
|---|---|---|
| magnesium | Mg | 4127g±0.1g |
| Zinc | Zn | 784g±0.1g |
| magnesium yttrium interalloy | Mg₈₉Y₁₁ | 571g±0.1g |
| boron carbide | B₄C | 300g±0.1g |
| zinc oxide | ZnO | 80g±1g |
| talcum powder | Mg₃[Si₄O₁₀](OH)₂ | 50g±1g |
| water glass | Na₂SiO₃·9H₂O | 25g±1g |
| deionized water | H₂O | 1000mL±50mL |
| aluminum foil | Al | 300mm×0.5mm×300mm |
| absolute alcohol | C₂H₅OH | 3500mL ±50mL |
| argon | Ar | 800000cm³±100 cm³ |
the preparation method comprises:
(1) preparing the casting mold
the open-close type squeeze casting mold is manufactured by hot working dies steel with a rectangle cavity, wherein the size of the cavity is 200mm×160mm×90mm and the surface roughness of the cavity is Ra 0.08-0.16µm;
(2) preparing the coating agent
weighing out zinc oxide 80g±1g, talcum powder 50g±1g, water glass 25g±1g, measuring out deionized water 300mL±1mL, adding zinc oxide 80g±1g, talcum powder 50g±1g, water glass 25g+1g and deionized water 300mL±1mL into the mixinghollander and stirring them to obtain the coating agent presenting as viscous liquid, wherein the stirring speed is 50r/min, stirring time is 80min;
(3) pre-treating the boron carbide particles
①ball milling: weighing boron carbide 300g±0.1g, putting it into the ball mill tank of the ball mill and ball milling it to obtain fine powder with a particle size ≤9µm, wherein the ball milling speed is 80r/min, the ball milling time is 3h;
②ultrasonic dispersion washing: putting the fine powder after ball milling into a beaker and then adding absolute alcohol 500mL±1mL, mixing;
putting the beaker into an ultrasonic disperser and doing the ultrasonic dispersion washing to obtain the mixing liquid, wherein the ultrasonic frequency is 60kHz and the ultrasonic dispersion time is 80min;
③filtration: putting the mixing liquid into the cloth funnel of the filter bottle, filtering it with a microporous membrane, removing the supernatant, and keeping the filter cake;
④drying and oxidation treatment: putting the filter cake into the thermal treatment furnace, conducting the drying and high temperature oxidation treatment, obtaining the boron carbide fine powderafter drying, wherein the drying and oxidation temperature is 500°C and the drying and oxidation time is 2h;
(4)pre-treating the magnesium, zinc and magnesium yttrium interalloy and the open-close type squeeze casting mold
①mechanically cutting the magnesium, zinc and magnesium yttrium interalloy into patches, wherein the size of the patch is ≤30mm×30mm×10mm;
②washing the surface of the magnesium, zinc and magnesium yttrium interalloy with absolute alcohol and then putting it into the vacuum drying oven after washing, wherein the drying temperature is 100°C, the vacuum degree is 2 Pa and the drying period is 30min;
③wrapping the boron carbide with aluminum foil, putting it into the vacuum drying ovenand drying, wherein the drying temperature is 100°C, the vacuum degree is 2 Pa and the drying period is 60min;
pre-heating the open-close type squeeze casting mold and coating the prepared coating agent on the inner surface of the mold cavity, wherein the thickness of the coating agent is 1mm; after the coating is completed, putting the open-close type squeeze casting mold into the heating furnace and preheating, wherein the pre-heating temperature is 150°C and the pre-heating time is 1h;
(5) smelting of the magnesium alloy
smelting of the magnesium alloy is conducted in the vacuum medium frequency induction melting furnace and completed by processes of medium frequency induction heating, vacuumizing, bottom blowing argon and mechanical stirring;
①opening the vacuum medium frequency induction melting furnace and clearing the internal part of the graphite melting crucible to make the internal part of the crucible clean;
②weighing magnesium block 4127g±0.1g, zinc block 784g±0.1g and magnesium yttrium interalloy block 571g±0.1g and putting them in the bottom of the crucible;
③closing the vacuum medium frequency induction melting furnace and getting it sealed;
turning on the vacuum pump and extracting the air within to allow the pressure within the furnace to reach 1Pa;
turning on the heater of the medium frequency induction melting furnace to start the heating, wherein the heating temperature is 610°C±1°C;
④turning on the argon bottom-blowing device to feed argon into the crucible, wherein the speed of the argon bottom-blowing is 200cm³/min; adjusting the pressure within the furnace to allow the pressure within the furnace to be one bar pressure and it is regulated by the outlet valve;
⑤when the temperature of melt is 610°C±1°C, adding boron carbide fine powder with the vacuum feeding device; turning on the mechanical agitator, wherein the stirring speed is 20r/min and the stirring time is 10min;
⑥stopping the stirring and continuing the heating; when the temperature of melt reaches 730°C±1°C, turning off the mechanical agitator and the argon bottom blowing pipe, standing for 10 min and prepare for the casting;
(6) squeeze casting
①opening the vacuum medium frequency induction melting furnace, removing the slag on the surface of the melt in the crucible, casting the alloy melt into the cavity of the squeeze casting mold; turning on the squeeze casting machine and squeezing the metal melt by the punch, wherein the squeeze pressure is 250MPa and the hold time is 20s;
the alloying reaction occurs during the solidification of Mg-Zn-Y quascicrystal and stable quascicrystal Mg₃Zn₆Y phase can be produced, wherein the reaction formula is $Mg + Zn + {Mg}_{89} {Y}_{11} + {B}_{4} C {\to }_{250 MPa}^{20 s} α - Mg + {Mg}_{3} {Zn}_{6} Y + {B}_{4} C$
α-Mg : substrate magnesium phase
Mg₃Zn₆Y : magnesium-zinc-yttrium quasicrystalline phase
②ejecting the cast and cooling it to 25°C in the air to produce the magnesium-zinc-yttrium quasicrystal and boron carbide mixed reinforced Mg-based composite material blocks;
(7)thermal treatment of the cast
①putting the magnesium-zinc-yttrium quasicrystal and boron carbide mixed reinforced Mg-based composite material blocks into the vacuum heat treatment furnace for thermal treatment, wherein the temperature of the thermal treatment is 420°C, the vacuum degree is 2Pa, and the time of thermal treatment is 15h; and then putting the cast into warm water of 50°C fastly, quenching treatment, wherein the quenching time is 20s;
②putting the cast after quenching into the heat treatment furnace for aging treatment at 200°C for 8h; and then stopping the heating and cooling it to 25°C in the heat treatment furnace;
(8) cleaning, detecting, analyzing and characterizing
cleaning the surface of the cast to make it clean; detecting, analyzing and characterizing the microstructure and mechanical property;
analyzing the metallographic structure with an optical microscope;
conducting the tensile strength and hardness test with universal tensile testing machine and a hardness tester;
conducting the fracture morphology analysis with a scanning electron microscope;
conducting XRD analysis with X ray diffractometer;
conclusion: magnesium-zinc-yttrium quasicrystal and boron carbide mixed reinforced Mg-based composite materials are rectangle blocks, wherein the tensile strength is 315MPa, the elongation is 7%, the hardness reaches 108Hv.

2. The method of preparing magnesium-zinc-yttrium quasicrystal and boron carbide mixed reinforced Mg-based composite materials according to claim 1, **characterized in that** the smelting of Mg-based composite materials are conducted in the vacuum medium frequency induction melting furnace and completed through the process of the medium frequency induction heating, bottom blowing argon and mechanical stirring;
the vacuum medium frequency induction melting furnace is a vertical one;
The bottom of the vacuum medium frequency induction melting furnace (1) is nconfigured with a furnace base (2), and inside of the vacuum medium frequency induction melting furnace (1) is a furnace chamber (3); a worktable (6) is configured in the bottom of the furnace chamber (3) and a graphite melting crucible (7) is put on the worktable (6); The outside of the graphite melting crucible (7) is surrounded by the medium frequency induction heater (8) and the inside of the graphite melting crucible (7) is the alloy melt (9); an outlet pipe (4) is configured on the top right of the vacuum medium frequency induction melting furnace (1) and it is controlled by the outlet valve (5); the argon bottle (15) is configured on the top left of the vacuum medium frequency induction melting furnace (1) and an argon pipe (16) and an argon valve (17) are configured on the argon bottle (15). The argon pipe (16) is connected to the bottom blow motor (11). The bottom blow motor (11) is connected to the bottom blow pipe (12). The bottom blow pipe (12) communicates to the graphite melting crucible (7) through the furnace base(2) and worktable (6) and bottom blows the alloy melt (9); a vacuum pump (13) is configured in the bottom right of the furnace base (2) and communicates to the furnace chamber (3) through a vacuum pipe (14); a feed pipe (27), a feed valve (28) and a mechanical agitator (29) are configured on the top of the vacuum medium frequency induction melting furnace (1) and the feed pipe (27) and the mechanical agitator (29) extends to the graphite melt crucible (7) through the furnace top base;
a electric cabinet (18) is configured on the right of the vacuum medium frequency induction melting furnace (1) and a display screen (19), an indicator light (20), a power switch (21), a medium frequency induction heating controller (22), a bottom blow motor controller (23) and a vacuum pump controller (24) are configured on the electric cabinet (18); the electric cabinet (18) is connected to the medium frequency induction heater (8) through a first cable (25); The electric cabinet (18) is connected to the bottom blow motor (11) and a vacuum pump (13) through the second cable (26); the furnace cavity (3) is filled with argon (10).

## Patentansprüche

1. Verfahren zum Herstellen eines gemischten verstärkten Verbundwerkstoffs auf Magnesiumbasis aus einem Magnesium-Zink-Yttrium-Quasikristall und Borcarbid, **dadurch gekennzeichnet, dass** die verwendeten chemische Materialien sind: Magnesium, Zink, Magnesium-Yttrium-Zwischenlegierung, Borcarbid, Zinkoxid, Talkumpuder, Wasserglas, das Na₂SiO₃·9H₂O ist, entionisiertes Wasser, Aluminiumfolie, reiner Alkohol, Argon, wobei deren Mengen sind:
| | | |
|---|---|---|
| Magnesium | Mg | 4127 g ± 0.1g |
| Zink | Zn | 784 g ± 0.1 g |
| Magnesium-Yttrium-Zwischenlegierung | Mg₈₉Y₁₁ | 571 g ± 0.1 g |
| Borcarbid | B₄C | 300 g ± 0.1 g |
| Zinkoxid | ZnO | 80 g ± 1 g |
| Talkumpuder | Mg₃[Si₄O₁₀(OH)₂ | 50g ± 1 g |
| Wasserglas | Na₂SiO₃·9H₂O | 25 g ± 1 g |
| entionisiertes Wasser | H₂O | 1000 ml ± 50 ml |
| Aluminiumfolie | Al | 300 mm × 0.5 mm × 300 mm |
| reiner Alkohol | C₂H₅OH | 3500 ml ± 50 ml |
| Argon | Ar | 800000 cm³ ± 100 cm³ |
wobei das Herstellungsverfahren aufweist:
(1) Herstellen einer Gießform
wobei eine öffnungs- und schließfähige Pressgießform durch Warmbearbeiten von Matrizenstahl mit einem rechteckigen Hohlraum hergestellt wird, wobei die Größe des Hohlraums 200 mm × 160 mm × 90 mm beträgt und die Oberflächenrauheit des Hohlraums Ra 0,08-0,16 µm beträgt;
(2) Herstellen eines Beschichtungsmittels
Abwiegen von Zinkoxid 80 g ± 1 g, Talkumpuder 50 g ± 1 g, Wasserglas 25 g ± 1 g, Abmessen von entionisiertem Wasser 300 ml ± 1 ml, Zugeben von Zinkoxid 80 g ± 1 g, Talkumpuder 50 g ± 1 g, Wasserglas 25 g ± 1 g und entionisiertem Wasser 300 ml ± 1 ml in einen Mischholländer und deren Rühren, um das Beschichtungsmittel zu erhalten, das als viskose Flüssigkeit vorliegt, wobei die Rührgeschwindigkeit 50 U/min beträgt und die Rührzeit 80 min beträgt;
(3) Vorbehandeln der Borcarbidteilchen
① Kugelmahlen: Abwiegen von Borcarbid 300 g ± 0,1 g, Geben desselben in den Kugelmühlentank der Kugelmühle und Kugelmahlen desselben, um ein feines Pulver mit einer Teilchengröße ≤ 9 µm zu erhalten, wobei die Kugelmahlgeschwindigkeit 80 U/min beträgt und die Kugelmahlzeit 3 h beträgt;
② Ultraschalldispersionswaschen: Geben des feinen Pulvers nach dem Kugelmahlen in ein Becherglas und dann Zugeben von reinem Alkohol 500 ml ± 1 ml, Mischen;
Setzen des Becherglases in eine Ultraschalldispersionsvorrichtung und Durchführen des Ultraschalldispersionswaschens, um die Mischflüssigkeit zu erhalten, wobei die Ultraschallfrequenz 60 kHz beträgt und die Ultraschalldispersionszeit 80 min beträgt;
③ Filtration: Geben der Mischflüssigkeit in einen Stofftrichter einer Filterflasche, Filtern desselben mit einer mikroporösen Membran, Entfernen des Überstands und Aufbewahren des Filterkuchens;
④ Trocknung und Oxidationsbehandlung: Geben des Filterkuchens in den Wärmebehandlungsofen, Durchführen der Trocknung und der Hochtemperaturoxidationsbehandlung, Erhalten des feinen Borcarbidpulvers nach der Trocknung, wobei die Trocknungs- und Oxidationstemperatur 500°C beträgt und die Trocknungs- und Oxidationszeit 2 h beträgt;
(4) Vorbehandeln des Magnesiums, des Zinks und der Magnesium-Yttrium-Zwischenlegierung und der öffnungs- und schließfähigen Pressgießform
① mechanisches Schneiden des Magnesiums, des Zinks und der Magnesium-Yttrium-Zwischenlegierung in Stücke, wobei die Größe des Stücks < 30 mm × 30 mm × 10 mm ist;
② Waschen der Oberfläche des Magnesiums, des Zinks und der Magnesium-Yttrium-Zwischenlegierung mit reinem Alkohol und Geben derselben in den Vakuumtrocknungsofen nach dem Waschen, wobei die Trocknungstemperatur 100°C beträgt, der Vakuumgrad 2 Pa beträgt und die Trocknungszeit 30 min beträgt;
③ Einwickeln des Borcarbids mit Aluminiumfolie, Geben desselben in den Vakuumtrocknungsofen und Trocknen, wobei die Trocknungstemperatur 100°C beträgt, der Vakuumgrad 2 Pa beträgt und die Trocknungszeit 60 min beträgt;
Vorheizen der öffnungs- und schließfähigen Pressgießform und Beschichten des hergestellten Beschichtungsmittels auf die Innenfläche des Formhohlraums, wobei die Dicke des Beschichtungsmittels 1 mm beträgt; nachdem das Beschichten beendet ist, Geben der öffnungs- und schließfähigen Pressgießform in den Heizofen und Vorheizen, wobei die Vorheiztemperatur 150°C beträgt und die Vorheizzeit 1 h beträgt;
(5) Schmelzen der Magnesiumlegierung
wobei das Schmelzen der Magnesiumlegierung in einem Vakuum-Mittelfrequenz-Induktionsschmelzofen durchgeführt wird und durch die Prozesse des Mittelfrequenz-Induktionserwärmung, Absaugens, des Bodeneinblasens von Argon und des mechanischen Rührens beendet wird;
① Öffnen des Vakuum-Mittelfrequenz-Induktionsschmelzofens und Leeren des Innenteils des Graphitschmelztiegels, um den Innenteil des Tiegels zu reinigen;
② Abwiegen eines Magnesiumblocks 4127 g ± 0,1 g, eines Zinkblocks 784 g ± 0,1 g und eines Magnesium-Yttrium-Zwischenlegierungsblocks 571 g ± 0,1 g und Geben derselben auf den Boden des Tiegels;
③ Schließen des Vakuum-Mittelfrequenz-Induktionsschmelzofen und Halten desselben geschlossen;
Einschalten der Vakuumpumpe und Absaugen der Luft darin, um den Druck im Ofen 1 Pa erreichen zu lassen;
Einschalten der Heizung des Mittelfrequenz-Induktionsschmelzofens, um die Erwärmung zu starten, wobei die Erwärmungstemperatur 610°C ± 1°C beträgt;
④ Einschalten der Argon-Bodenblasvorrichtung, um Argon in den Tiegel zuzuführen, wobei die Geschwindigkeit des Argon-Bodenblasens 200 cm³/min beträgt; Einstellen des Drucks im Ofen, um den Druck im Ofen auf ein 1 Bar Druck zu bringen, der durch ein Auslassventil geregelt wird;
⑤ wenn die Temperatur der Schmelze 610°C ± 1°C beträgt, Zugeben des feinen Borcarbidpulvers mit einer Vakuumzufuhrvorrichtung; Einschalten des mechanischen Rührers, wobei die Rührgeschwindigkeit 20 U/min beträgt und die Rührzeit 10 min beträgt;
⑥ Stoppen des Rührens und Fortsetzen des Erwärmens; wenn die Temperatur der Schmelze 730°C ± 1°C erreicht, Abschalten des mechanischen Rührers und einer Argon-Bodenblasleitung, Stehenlassen für 10 min und Vorbereiten des Gießens;
(6) Pressgießen
① Öffnen des Vakuum-Mittelfrequenz-Induktionsschmelzofens, Entfernen der Schlacke auf der Oberfläche der Schmelze im Tiegel, Gießen der Legierungsschmelze in den Hohlraum der Pressgießform; Einschalten der Pressgießmaschine und Pressen der Metallschmelze durch einen Stempel, wobei der Pressdruck 250 MPa beträgt und die Haltezeit 20 s beträgt;
die Legierungsreaktion tritt während der Verfestigung des Mg-Zn-Y-Quasikristalls auf, und es kann eine stabile Quasikristall-Mg₃Zn₆Y-Phase erzeugt werden, wobei die Reaktionsformel ist $Mg + Zn + {Mg}_{89} {Y}_{11} + {B}_{4} C {\to }_{250 MPa}^{20 s} α - Mg + {Mg}_{3} {Zn}_{6} Y + {B}_{4} C$
α-Mg : Substratmagnesiumphase
Mg₃Zn₆Y : Magnesium-Zink-Yttrium-Quasikristall-Phase
② Auswerfen des Gusses und dessen Abkühlung auf 25°C in der Luft, um die gemischten verstärkten Verbundwerkstoffblöcke auf Magnesiumbasis aus Magnesium-Zink-Yttrium-Quasikristall und Borcarbid zu erzeugen;
(7) Wärmebehandeln des Gusses
① Geben der gemischten verstärkten Verbundwerkstoffblöcke auf Magnesiumbasis aus Magnesium-Zink-Yttrium-Quasikristall und Borcarbid in einen Vakuum-Wärmebehandlungsofen zum Wärmebehandeln, wobei die Temperatur der Wärmebehandlung 420°C beträgt, der Vakuumgrad 2 Pa beträgt und die Zeit der Wärmebehandlung 15 h beträgt; und dann schnelles Geben des Gusses in warmes Wasser mit 50°C, Abschreckbehandlung, wobei die Abschreckzeit 20 s beträgt;
② Geben des Gusses nach dem Abschrecken in den Wärmebehandlungsofen zur Alterungsbehandlung bei 200°C für 8h; und dann Stoppen der Erwärmung und der Abkühlung auf 25°C im Wärmebehandlungsofen;
(8) Reinigen, Erfassen, Analysieren und Charakterisieren
Reinigen der Oberfläche des Gusses, um ihn zu reinigen; Erfassen, Analysieren und Charakterisieren des Mikrogefüges und der mechanischen Eigenschaft;
Analysieren des metallographischen Gefüges mit einem optischen Mikroskop; Durchführen einer Zugfestigkeits- und Härteprüfung mit einer Universalzugprüfmaschine und einem Härteprüfgerät;
Durchführen einer Analyse der Bruchmorphologie mit einem Rasterelektronenmikroskop;
Durchführen einer Röntgenbeugungsanalyse mit einem Röntgendiffraktometer; Schlussfolgerung: gemischten verstärkten Verbundwerkstoffe auf Magnesiumbasis aus Magnesium-Zink-Yttrium-Quasikristall und Borcarbid sind rechteckige Blöcke, wobei die Zugfestigkeit 315 MPa beträgt, die Dehnung 7% beträgt, die Härte 108 Hv erreicht.

2. Verfahren zum Herstellen eines gemischten verstärkten Verbundwerkstoffs auf Magnesiumbasis aus einem Magnesium-Zink-Yttrium-Quasikristall und Borcarbid nach Anspruch 1, **dadurch gekennzeichnet, dass** das Schmelzen des Verbundwerkstoffs auf Magnesiumbasis in einem Vakuum-Mittelfrequenz-Induktionsschmelzofen durchgeführt wird und durch den Prozess der Mittelfrequenz-Induktionserwärmung, des Bodeneinblasens von Argon und des mechanischen Rührens beendet wird;
der Vakuum-Mittelfrequenz-Induktionsschmelzofen ein vertikaler ist;
der Boden des Vakuum-Mittelfrequenz-Induktionsschmelzofens (1) mit einer Ofenbasis (2) konfiguriert ist, und das Innere des Vakuum-Mittelfrequenz-Induktionsschmelzofens (1) eine Ofenkammer (3) ist; ein Arbeitstisch (6) am Boden der Ofenkammer (3) konfiguriert ist und ein Graphitschmelztiegel (7) auf den Arbeitstisch (6) gestellt wird; das Äußere des Graphitschmelztiegels (7) durch die Mittelfrequenz-Induktionsheizung (8) umgeben ist und das Innere des Graphitschmelztiegels (7) die Legierungsschmelze (9) ist; eine Auslassleitung (4) auf der oberen rechten Seite des Vakuum-Mittelfrequenz-Induktionsschmelzofens (1) konfiguriert ist und durch das Auslassventil (5) gesteuert wird; eine Argonflasche (15) auf der oberen linken Seite des Vakuum-Mittelfrequenz-Induktionsschmelzofens (1) konfiguriert ist und eine Argonleitung (16) und ein Argonventil (17) an der Argonflasche (15) konfiguriert sind; die Argonleitung (16) mit einem Bodenblasmotor (11) verbunden ist; der Bodenblasmotor (11) mit einer Bodenblasleitung (12) verbunden ist; die Bodenblasleitung (12) durch die Ofenbasis (2) und den Arbeitstisch (6) mit dem Graphitschmelztiegel (7) in Verbindung steht und die Legierungsschmelze (9) bodenbläst; eine Vakuumpumpe (13) an der unteren rechten Seite der Ofenbasis (2) konfiguriert ist und durch eine Vakuumleitung (14) mit der Ofenkammer (3) in Verbindung steht; eine Zufuhrleitung (27), ein Zufuhrventil (28) und ein mechanischer Rührer (29) auf dem Vakuum-Mittelfrequenz-Induktionsschmelzofen (1) konfiguriert sind und sich die Zufuhrleitung (27) und der mechanische Rührer (29) durch die obere Ofenbasis zum Graphitschmelztiegel (7) erstrecken;
ein Schaltschrank (18) auf der rechten Seite des Vakuum-Mittelfrequenz-Induktionsschmelzofens (1) konfiguriert ist und ein Anzeigebildschirm (19), eine Anzeigelampe (20), ein Stromschalter (21), eine Mittelfrequenz-Induktionserwärmungssteuerung (22), eine Bodenblasmotorsteuerung (23) und eine Vakuumpumpensteuerung (24) im Schaltschrank (18) konfiguriert sind; der Schaltschrank (18) mit der Mittelfrequenz-Induktionsheizung (8) durch ein erstes Kabel (25) verbunden ist; der Schaltschrank (18) mit dem Bodenblasmotor (11) und der Vakuumpumpe (13) durch ein zweites Kabel (26) verbunden ist; der Ofenhohlraum (3) mit Argon (10) gefüllt ist.

## Revendications

1. Procédé de préparation de matériaux composites à base de Mg renforcés par mélange de quasi-cristaux magnésium-zinc-yttrium et de carbure de bore, **caractérisé en ce que** les matériaux chimiques utilisés sont : magnésium, zinc, alliage magnésium-yttrium, carbure de bore, oxyde de zinc, poudre de talc, verre soluble étant une eau déminéralisée Na₂SiO₃·9H₂O, papier d'aluminium, alcool pur, argon, avec les teneurs suivantes :
| | | |
|---|---|---|
| magnésium | Mg | 4127 g ± 0,1 g |
| zinc | Zn | 784 g ± 0,1 g |
| alliage magnésium-yttrium | Mg₈₉Y₁₁ | 571 g ± 0,1 g |
| carbure de bore | B₄C | 300 g ± 0,1 g |
| oxyde de zinc | ZnO | 80 g ± 1 g |
| poudre de talc | Mg₃[Si₄O₁₀](OH)₂ | 50 g ± 1 g |
| verre soluble | Na₂SiO₃·9H₂O | 25 g ± 1 g |
| eau déminéralisée | H₂O | 1000 ml ± 50 ml |
| papier d'aluminium | Al | 300 mm × 0,5 mm × 300 mm |
| alcool pur | C₂H₅OH | 3500 ml ± 50 ml |
| argon | Ar | 800000 cm³ ± 100 cm³ |
ledit procédé de préparation comprenant :
(1) la préparation du moule de coulée
le moule de coulée sous pression de type fermé-ouvert est fabriqué par usinage à chaud d'acier à matrices avec une cavité rectangulaire, la cavité ayant une grandeur de 200 mm × 160 mm × 90 mm et la rugosité de surface Ra de la cavité étant comprise entre 0,08 et 0,16 µm ;
(2) la préparation de l'agent de revêtement
pesée d'oxyde de zinc 80 g ± 1 g, de poudre de talc 50 g ± 1 g, de verre soluble 25 g ± 1 g, mesure d'eau déminéralisée 300 ml ± 1 ml, ajout d'oxyde de zinc 80 g ± 1 g, de poudre de talc 50 g ± 1 g, de verre soluble 25 g ± 1 g et d'eau déminéralisée 300 ml ± 1 ml dans le malaxeur Hollander et agitation afin d'obtenir l'agent de revêtement se présentant sous forme de liquide visqueux, la vitesse d'agitation étant de 50r/min, le temps d'agitation de 80 min ;
(3) pré-traitement des particules de carbure de bore
① broyage à billes : pesée de carbure de bore 300 g ± 0,1 g, mis en place dans le réservoir du broyeur à billes, et soumis à un broyage à billes afin d'obtenir une poudre fine ayant une granulométrie ≤ 9 µm, la vitesse de broyage à billes speed étant de 80r/min, le temps de broyage à billes de 3 h ;
② lavage à dispersion ultrasonique : après le broyage à billes, versement de la poudre fine dans un bécher et ajout d'alcool pur 500 ml ± 1 ml, mélange ;
mise en place du bécher dans un disperseur ultrasonique et exécution du lavage à dispersion ultrasonique afin d'obtenir le liquide de mélange, la fréquence ultrasonore étant de 60 kHz et le temps de dispersion ultrasonique de 80 min ;
③ filtration : versement du liquide de mélange dans la cheminée de tissu de la bouteille filtrante, filtration par membrane microporeuse, retrait du surnageant, et conservation du gâteau de filtration ;
④ traitement de séchage et d'oxydation : mise en place du gâteau de filtration dans le four de traitement thermique, application du traitement de séchage et d'oxydation à haute température, obtention de la poudre fine de carbure de bore après séchage, la température de séchage et d'oxydation étant de 500 °C et le temps de séchage et d'oxydation de 2 h ;
(4) pré-traitement du magnésium, du zinc et de l'alliage magnésium-yttrium et du moule de coulée sous pression de type fermé-ouvert
① découpe mécanique en pièces du magnésium, du zinc et de l'alliage magnésium-yttrium, la grandeur de pièce étant ≤ 30 mm × 30 mm × 10 mm ;
② lavage de surface par alcool pur du magnésium, du zinc et de l'alliage magnésium-yttrium et mise en place dans le four de séchage sous vide après lavage, la température de séchage étant de 100 °C, le degré de vide de 2 Pa et la durée de séchage de 30 min ;
③ emballage du carbure de bore avec du papier d'aluminium, mise en place dans le four de séchage sous vide et séchage, la température de séchage étant de 100 °C, le degré de vide de 2 Pa et la durée de séchage de 60 min ;
pré-chauffage du moule de coulée sous pression de type fermé-ouvert et revêtement de la surface intérieure de la cavité de moule par l'agent de revêtement préparé, l'épaisseur de l'agent de revêtement étant de1mm ; à l'issue du revêtement, mise en place du moule de coulée sous pression de type fermé-ouvert dans le four de chauffage et pré-chauffage, la température de pré-chauffage étant de 150 °C et le temps de pré-chauffage de 1 h ;
(5) fusion de l'alliage de magnésium
la fusion de l'alliage de magnésium est exécutée dans le four de fusion par induction à fréquence moyenne sous vide et terminée par processus de chauffage par induction à fréquence moyenne, mise sous vide, soufflage d'argon par le fond et agitation mécanique,
① ouverture du four de fusion par induction à fréquence moyenne sous vide et nettoyage de la partie intérieure du creuset de fusion en graphite pour rendre propre la partie intérieure du creuset ;
② pesée d'un bloc de magnésium de 4127 g ± 0,1 g, d'un bloc de zinc de 784 g ± 0,1 g et d'un bloc d'alliage magnésium-yttrium de 571 g ± 0,1 g, et mise en place de ceux-ci au fond du creuset ;
③ fermeture du four de fusion par induction à fréquence moyenne sous vide et verrouillage de celui-ci ;
activation de la pompe à vide et extraction de l'air intérieur pour que la pression à l'intérieur du atteigne 1 Pa ;
activation du chauffage du four de fusion par induction à fréquence moyenne pour commencer le chauffage, la température de chauffage étant de 610 °C ± 1 °C ;
④ activation du dispositif de soufflage d'argon par le fond pour alimenter le creuset en argon, la vitesse de soufflage d'argon par le fond étant de 200cm³/min ; réglage de la pression à l'intérieur du four pour porter à un bar la pression à l'intérieur du four et régulation par la vanne de sortie ;
⑤ si la température de fusion est de 610 °C ± 1 °C, ajout de poudre fine de carbure de bore par le dispositif d'alimentation à vide ; activation de l'agitateur mécanique, la vitesse d'aspiration étant de 20r/min et le temps d'agitation de 10 min ;
⑥ arrêt de l'agitation et poursuite du chauffage ; si la température de fusion atteint 730 °C ± 1 °C, désactivation de l'agitateur mécanique et du conduit de soufflage d'argon par le fond, durée de repos 10 min et préparation pour la coulée ;
(6) coulée sous pression
① ouverture du four de fusion par induction à fréquence moyenne sous vide, retrait des scories à la surface de la fonte dans le creuset, coulée de l'alliage fondu dans la cavité du moule de coulée sous pression ; activation de la machine à couler sous pression et compression du métal fondu par le poinçon, la pression étant de 250 MPa et le temps de maintien de 20 s ;
la réaction d'alliage survenant pendant la solidification des quasi-cristaux Mg-Zn-Y est $Mg + Zn + {Mg}_{89} {Y}_{11} + {B}_{4} C {\to }_{250 MPa}^{20 s} α - Mg + {Mg}_{3} {Zn}_{6} Y + {B}_{4} C$
une phase quasi-cristalline Mg3Zn6Y stable pouvant être obtenue, la formule de réaction étant
α-Mg: phase de substrat magnésium
Mg₃Zn₆Y : phase quasi-cristalline magnésium-zinc-yttrium
② éjection du moulage et refroidissement à l'air à 25 °C pour produire les quasi-cristaux magnésium-zinc-yttrium et les blocs de matériau composite à base de Mg renforcés par mélange de carbure de bore ;
(7) traitement thermique du moulage
① chargement pour traitement thermique des quasi-cristaux magnésium-zinc-yttrium et des blocs de matériau composite à base de Mg renforcés par mélange de carbure de bore dans le four de traitement thermique sous vide, la température du traitement thermique étant de 420 °C, le degré de vide de 2 Pa, et le temps de traitement thermique de 15 h ; puis trempage rapide du moulage dans l'eau chaude à 50 °C, traitement de trempe, le temps de trempe étant de 20 s ;
② mise en place du moulage dans le four de traitement thermique après trempe pour traitement de vieillissement à 200 °C pendant 8 h ; puis arrêt du chauffage et refroidissement à 25 °C dans le four de traitement thermique ;
(8) nettoyage, détection, analyse et caractérisation
nettoyage de la surface du moulage pour le rendre propre ; détection, analyse et caractérisation de la microstructure et des propriétés mécaniques ;
analyse de la structure métallographique avec un microscope optique ;
essai de résistance à la traction et de dureté avec une machine d'essai de traction universelle et un testeur de dureté ;
analyse de morphologie de fracture avec un microscope électronique à balayage ; analyse XRD avec un diffractomètre à rayon X ;
conclusion : les quasi-cristaux magnésium-zinc-yttrium et les matériaux composites à base de Mg renforcés par mélange de carbure de bore sont des blocs rectangulaires, la résistance à la traction étant de 315 MPa, l'allongement de 7 %, la dureté atteignant 108 Hv.

2. Procédé de préparation de matériaux composites à base de Mg renforcés par mélange de quasi-cristaux magnésium-zinc-yttrium et de carbure de bore selon la revendication 1, **caractérisé en ce que** la fusion des matériaux composites à base de Mg est exécutée dans le four de fusion par induction à fréquence moyenne sous vide et terminée par processus de chauffage par induction à fréquence moyenne, soufflage d'argon par le fond et agitation mécanique ;
le four de fusion par induction à fréquence moyenne sous vide est un four vertical ;
le fond du four de fusion par induction à fréquence moyenne sous vide (1) est prévu avec une base de four (2), et à l'intérieur du four de fusion par induction à fréquence moyenne sous vide (1), une chambre de four (3) ; une table de travail (6) est prévue au fond de la chambre de four (3) et un creuset de fusion en graphite (7) est disposé sur la table de travail (6) ; l'extérieur du creuset de fusion en graphite (7) est entouré par le chauffage par induction à fréquence moyenne (8) et l'intérieur du creuset de fusion en graphite (7) contient l'alliage fondu (9) ; un conduit de sortie (4) est prévu en haut à droite du four de fusion par induction à fréquence moyenne sous vide (1) et est commandé par la vanne de sortie (5) ; la bouteille d'argon (15) est prévue en haut à gauche du four de fusion par induction à fréquence moyenne sous vide (1) et un conduit d'argon (16) ainsi qu'une vanne à argon (17) sont prévus sur la bouteille d'argon (15) ; le conduit d'argon (16) est relié au moteur de soufflage par le fond (11) ; le moteur de soufflage par le fond (11) est relié au conduit de soufflage par le fond (12) ; le conduit de soufflage par le fond (12) communique avec le creuset de fusion en graphite (7) en traversant la base de four (2) et la table de travail (6), et souffle par le fond l'alliage fondu (9) ; une pompe à vide (13est prévue en bas à droite de la base de four (2) et communique avec la chambre de four (3) par un conduit de vide (14) ; un conduit d'alimentation (27), une vanne d'alimentation (28) et un agitateur mécanique (29) sont prévus sur le dessus du four de fusion par induction à fréquence moyenne sous vide (1), et le conduit d'alimentation (27) et l'agitateur mécanique (29) s'étendent vers le creuset de fusion en graphite (7) en traversant la base supérieure du four ;
une armoire électrique (18) est prévue à droite du four de fusion par induction à fréquence moyenne sous vide (1) et un écran d'affichage (19), un voyant indicateur (20), un interrupteur (21), un dispositif de commande (22) du chauffage par induction à fréquence moyenne, un dispositif de commande (23) du moteur de soufflage par le fond et un dispositif de commande (24) de la pompe à vide sont prévus sur l'armoire électrique (18) ; l'armoire électrique (18) est reliée au chauffage par induction à fréquence moyenne (8) par un premier câble (25) ; l'armoire électrique (18) est reliée au moteur de soufflage par le fond (11) et à une pompe à vide (13) par le deuxième câble (26) ; la cavité du four (3) est remplie d'argon (10).
